

## 1

3,282,690  
ALLOY

Eugene J. Delgrosso, Wallingford, and John J. Kaminsky, Cromwell, Conn., assignors to United Aircraft Corporation, East Hartford, Conn., a corporation of Delaware  
No Drawing. Filed Dec. 2, 1963, Ser. No. 327,552  
5 Claims. (Cl. 75—174)

This invention relates to columbium-base alloys and methods of preparing them and has among its objects to provide a group of alloys which are attractive for use from room temperature to 2400° F. either as a structural member in the form of a rod, extrusion or large-size forging, or as tubing for conveying high temperature liquid metal; which are characterized by very high strength and creep resistance at 2400° F.—better than the best commercial columbium alloys available today; which have good fabricability, being capable of rolling to foil; and which possess corrosion resistance equal to that of electron beam produced Cb-1Zr.

These and other objects and advantages of the alloys of this invention will be evident from the following detailed description of a number of alloys and their properties which come within the scope of the invention.

This alloy family is intended for use up to 2400° F., which makes it very attractive for use in present nuclear reactors and it may well supplant the electron beam prepared Cb-1Zr currently used for reactor applications. On a strength to weight basis, the alloys of this invention are superior to most tantalum and tungsten base alloys at 2400° F.

The alloys of this invention consist of columbium, zirconium and carbon in the following proportions:

Cb-(1 to 8 w/o)Zr-(0.05—1.0 w/o)C

This series of alloys have been prepared and subjected to intensive mechanical properties evaluation. The concentrations of the alloying agents were varied in the following manners:

(a) The ratio of zirconium atoms to carbon atoms, at a fixed zirconium level, was varied to ascertain if any change in properties resulted from deviations from the atomic stoichiometry of one, i.e.,

Number of Zr atoms/number of C atoms=1

(b) In order to vary the phase size and phase concentration of carbides, the total zirconium and carbon contents were increased from the 1 w/o level to the 5 w/o level, while maintaining a constant zirconium to carbon atomic ratio of 1.

On the basis of this work, it was determined that best strength results are obtained when the zirconium to carbon atomic ratio is maintained approximately equal to one. The greatest strength improvements were obtained by increasing the zirconium and carbon concentrations to the 3 w/o and 0.5 w/o levels, respectively; beyond this concentration level, any additional strengthening was considered fairly marginal. The carbon additions were not found to be detrimental to the fabricability of worked material, whereas oxygen and nitrogen were detrimental to the ductility of even wrought Cb-Zr alloys. Furthermore, experimentation with a series of Cb-Zr alloys doped with oxygen and/or nitrogen revealed that little strengthening was produced at 2400° F., hence oxygen and nitrogen are considered undesirable constituents to the Cb-Zr-C alloy and every effort is exerted to reduce the level of these interstitials.

## 2

The preferred compositions for this family of alloys are:

Cb-1 Zr-0.1 C, Cb-3 Zr-0.35 C

5 The carbon levels are rigidly controlled to within  $\pm 10\%$  of the desired composition in order to achieve reproducibility of properties. In addition, high purity columbium base metal is utilized to maintain low oxygen and nitrogen levels in the alloy.

10 Information about the properties and behavior of these alloys was generated in the following areas:

(1) *Melting*.—Suitable alloys were prepared by non-consumable and consumable arc melting techniques, as well as by employment of electron beam melting. Dense 15 electrodes for melting were prepared by compaction of blended mixtures of powders, followed by sintering in vacuum at 2200° F. for two hours. Careful preparation of the alloy charge is extremely important for the following reasons:

20 (a) Due to a Co boil in melting, carbon losses can be substantial; therefore, excess quantities of carbon, added as CbC, or Cb<sub>2</sub>C, must be added to the charge to properly compensate for losses.

(b) In general, two carbides can be formed in the alloy 25 and experimentation has indicated that the method of adding the carbon has an influence on the type of carbide formed as well as on the degree of alloying and segregation. It has been our experience that carbon should be added as a carbide rather than as elemental carbon to 30 achieve more rapid alloying with the metallic elements and a more uniform distribution. Generally the carbon is added as ZrC to whatever level of zirconium and carbon is desired, and excess carbon to counterbalance melting losses is added as CbC or Cb<sub>2</sub>C. Excess concentrations 35 vary from 5 to 25 w/o of the desired carbon level, depending upon the total carbon required and the melting technique utilized. Melting technique varies due to the fact that several arc furnaces are available for melting and such operating factors as power, vacuum level, ingot size and molten pool size are different for each furnace.

(2) *Fabrication*.—These Cb-Zr-C alloys are completely 40 fabricable under hot, warm and cold working conditions. The alloys were successfully extruded and/or forged at temperatures from 2200 to 3300° F.; wrought forms such 45 as rod, sheet, plate and tubing were successfully manufactured, as well as wire. In order to obtain optimum strengthening it is important to properly control warm and hot working operations to achieve proper solutioning and precipitation for both fine particle strengthening and 50 interaction of dislocation networks with fine particles for additional strengthening. The effect of cold working on elevated temperature strengthening has also been determined.

(3) *Heat Treatment*.—The heat treatment response of 55 several of the alloys, Cb-1 Zr-0.1 and Cb-3 Zr-0.3 C, has been thoroughly investigated with respect to stress relief annealing, recovery, recrystallization, grain growth and aging. This work indicated cold worked material could be stress relief annealed by heating for 1 to 2 hours in 60 vacuum at 2400° F. Also, recrystallization and grain growth occurred at 2900° F. or higher and generally was associated with the solutionizing of the carbide phase.

(4) *Phase and Structure Studies*.—A study has been 65 made of the carbide phases present in these alloys and the effect of heat treating on their composition and structure of these carbides. Particular attention has been paid to the Cb-3 Zr-0.3 C and Cb-1 Zr-0.1 C alloys. Two

carbides have been observed in these alloys under various experimental conditions:  $[(\text{CbZr})\text{C}]$  an alloyed form of cubic zirconium carbide and  $[(\text{CbZr})_2\text{C}]$  an alloyed form of hexagonal columbium carbide. Also, a detailed

can be restored in part or almost fully by recrystallizing the material to a fine grain size ASTM 7 to 8 and concomitantly precipitating very fine carbides in the grain boundaries.

TABLE I.—Cb-3 Zr-0.35 C Weld Data

## A. FUSION WELDED

| Test Configuration                  | Weld Condition                   | Results                             |
|-------------------------------------|----------------------------------|-------------------------------------|
| Specimen bent parallel to weld      | As welded                        | Limited ductility, bent thru 11°.   |
| Specimen bent parallel to weld      | Heat treated 2 hrs. at 2,200° F. | Limited ductility, bent thru 32°.   |
| Specimen bent perpendicular to weld | Heat treated 2 hrs. at 2,200° F. | Limited ductility, bent thru 29°.   |
| Specimen bent perpendicular to weld | Heat treated 1 hr. at 2,400° F.  | Limited ductility, bent thru 51°.   |
| Specimen bent parallel to weld      | Heat treated 1 hr. at 2,400° F.  | Complete ductility, bent thru 100°. |

## B. Cb-1 Zr FILLER WELD

|                                     |                                  |                                     |
|-------------------------------------|----------------------------------|-------------------------------------|
| Specimen bent parallel to weld      | As welded                        | Limited ductility, bent thru 10°.   |
| Specimen bent perpendicular to weld | As welded                        | Limited ductility, bent thru 15°.   |
| Specimen bent parallel to weld      | Heat treated 2 hrs. at 2,200° F. | Complete ductility, bent thru 114°. |
| Specimen bent perpendicular to weld | Heat treated 2 hrs. at 2,200° F. | Complete ductility, bent thru 22°.  |
| Specimen bent parallel to weld      | Heat treated 1 hr. at 2,400° F.  | Complete ductility, bent thru 110°. |
| Specimen bent perpendicular to weld | Heat treated 1 hr. at 2,400° F.  | Limited ductility, bent thru 29°.   |

TABLE II

TITLE: TENSILE STRENGTH DATA  
SUBTITLE: MATERIAL IN EXTRUDED CONDITION

| Alloy          | Test Temp. °F. | Yield Strength | Ultimate Tensile Strength | Percent Elongation | Percent Reduction in Area |
|----------------|----------------|----------------|---------------------------|--------------------|---------------------------|
| Cb-1 Zr-0.1 C  | R.T.           | 53,400         | 71,300                    | 25                 | 65                        |
| Cb-1 Zr-0.1 C  | 2,400          | 16,700         | 17,400                    | 24                 | 63                        |
| Cb-1 Zr-0.1 C  | 2,600          | 9,000          | 9,600                     | 27                 | 99                        |
| Cb-2 Zr-0.2 C  | 2,200          | 23,200         | 24,300                    | 13                 | 85                        |
| Cb-2 Zr-0.2 C  | 2,400          | 15,600         | 16,400                    | 15                 | 81                        |
| Cb-3 Zr-0.35 C | R.T.           | 89,600         | 122,900                   | 16                 | 31                        |
| Cb-3 Zr-0.35 C | 2,200          | 47,600         | >50,700                   | 8                  | 54                        |
| Cb-3 Zr-0.35 C | 2,400          | 22,500         | 23,500                    | 25                 | 90                        |
| Cb-3 Zr-0.35 C | 2,600          | 14,700         | 15,300                    | 27                 | 96                        |
| Cb-3 Zr-0.4 C  | R.T.           | 63,600         | 80,500                    | 19                 | 32                        |
| Cb-3 Zr-0.4 C  | 2,200          | 39,700         | 45,800                    | 14                 | 96                        |
| Cb-3 Zr-0.4 C  | 2,400          | 23,500         | 24,400                    | 23                 | 86                        |
| Cb-3 Zr-0.6 C  | 2,400          | 14,200         | 16,000                    | 18                 | 70                        |
| Cb-4 Zr-0.7 C  | 2,200          | 26,300         | 37,200                    | 15                 | 53                        |
| Cb-4 Zr-0.7 C  | 2,400          | 21,200         | 25,500                    | 12                 | 61                        |
| Cb-5 Zr-0.6 C  | 2,200          | 32,800         | 37,700                    | 9                  | 57                        |
| Cb-5 Zr-0.6 C  | 2,400          | 23,500         | 26,300                    | 10                 | 56                        |

electron transmission metallography study has been made of the grain structure and substructure of the Cb-3 Zr-0.3 C and Zb-1 Zr-0.1 C alloys. Particular attention has been paid to the dislocation characteristics of these alloys, and a theory of strengthening has been proposed on the basis of dislocation-dislocation and precipitate-dislocation interactions in these alloys.

(5) *Oxidation Resistance.*—The oxidation behavior of the Cb-3 Zr-0.3 C and Cb-1 Zr-0.1 C alloys was determined to be similar to that of CB-1 Zr from 1600 to 2200° F. in air.

(6) *Weldability.*—These alloys can be successfully fusion welded or welded with filler wire, made from Cb-1 Zr or the base metal itself. Sheets from 45 up to 100 mils thick have been successfully welded by both fusion and filler techniques. Welded alloy sheet material has been subjected to extensive bend testing, all tests conducted according to the standards of the Materials Advisory Board 4T test) and typical results for Cb-3 Zr-0.3 C are summarized in Table I. In the as-welded condition, the alloy was not brittle but possessed limited ductility; complete ductility was achieved by the appropriate annealing treatments listed in Table I.

(7) *Strength.*—The tensile strengths of the alloys were determined as a function of fabrication history and test temperature. These results are summarized in Table II. Creep rupture testing was concentrated on the Cb-3 Zr-0.35 C and Cb-1 Zr-0.1 C alloys. Results are presented in Table III. The greatest strength values in the Cb-3 Zr-0.3 C alloy were developed by warm extruding at 3050 to 3150° F. The influence of annealing, cold working and recrystallization upon the strength of the Cb-1 Zr-0.1 C and Cb-3 Zr-0.35 C has been delineated. In general, cold working causes a strength reduction which

45

TABLE III

TITLE: 100 HOUR STRESS TO RUPTURE DATA  
SUBTITLE: MATERIAL IN EXTRUDED CONDITION, TESTED IN VACUUM

| Alloy          | Test Temp. °F. | 100 Hour Stress Rupture Life, p.s.i. | Percent Elongation | Percent Reduction in Area |
|----------------|----------------|--------------------------------------|--------------------|---------------------------|
| Cb-1 Zr-0.1 C  | 2,200          | 13,500                               | —                  | —                         |
| Cb-1 Zr-0.1 C  | 2,400          | 7,000                                | 28                 | 96                        |
| Cb-2 Zr-0.2 C  | 2,400          | 4,500                                | 28                 | 95                        |
| Cb-3 Zr-0.35 C | 2,150          | 17,000                               | 4                  | 4                         |
| Cb-3 Zr-0.35 C | 2,400          | 13,000                               | 28                 | —                         |
| Cb-3 Zr-0.6 C  | 2,400          | 6,000                                | 35                 | 84                        |
| Cb-4 Zr-0.7 C  | 2,150          | 17,000                               | —                  | —                         |
| Cb-5 Zr-0.6 C  | 2,150          | 7,500                                | 34                 | 48                        |
| Cb-5 Zr-0.6 C  | 2,400          | 12,000                               | 27                 | 84                        |

<sup>1</sup> Test stopped; did not go to completion.

It will thus be evident that as a result of this invention improved columbium-base alloys have been provided and an improved method of making them, enabling large structural members and large-size forgings to be constructed which are capable of use from room temperature to 2400° F. as well as tubing for conveying high-temperature liquid metal from a reactor core, for example, to more remote parts of the reactor system.

It will further be evident that as a result of this invention improved columbium-base alloys have been provided having high strength and good creep resistance at 2400° F. and which have excellent fabricability and good corrosion resistance at this elevated temperature.

While our invention has been described by means of certain specific examples, it is to be understood that the scope of the invention is not to be limited thereby except as defined by the following claims.

50

60

65

70

75

We claim:

1. An article of manufacture having good strength, creep resistance, corrosion resistance and fabricability up to temperatures of about 2400° F. which consists essentially of, by weight, 1-8% zirconium, and 0.05-1% carbon, balance columbium having a low oxygen and nitrogen interstitial content.

2. An article of manufacture according to claim 1 in which the oxygen and nitrogen interstitial contents are, by weight, as follows, 0-150 p.p.m. oxygen and 0-200 p.p.m. nitrogen.

3. A columbium base alloy having high tensile strength and good creep resistance at 2400° F. which consists essentially of, by weight, about 1% zirconium and about 0.1% carbon, balance columbium.

4. A columbium base alloy having high tensile strength and good creep resistance at 2400° F. which consists essentially of, by weight, about 3% zirconium and about 0.35% carbon, balance columbium.

5. In the preparation of the columbium-zirconium-carbon alloys, the method of making the carbon addition to the alloy comprising the steps of, admixing high purity columbium and zirconium carbide in a weight ratio of

columbium to zirconium substantially equal to that desired in the cast alloy, adding excess carbon thereto in the form of a second carbide selected from that group of carbides consisting of CbC and Cb<sub>2</sub>C, the amount of carbon added in the second carbide equalling that lost in the melting process, and melting the mixture in a non-contaminating atmosphere.

References Cited by the Examiner

UNITED STATES PATENTS

10 3,056,672 10/1962 Clark ----- 75-174  
3,181,946 5/1965 McAndrew et al. ----- 75-174

FOREIGN PATENTS

15 915,416 1/1963 Great Britain.

OTHER REFERENCES

20 "Columbium-Base Alloys," Flight Propulsion Laboratory Department of the General Electric Co., February 1962, Cleveland, Ohio.

DAVID L. RECK, Primary Examiner.

C. N. LOVELL, Assistant Examiner.